

## 1

3,036,905

## MOTOR FUEL

Martin Hamer, Chicago, Ill., assignor to Standard Oil Company, Chicago, Ill., a corporation of Indiana  
No Drawing. Filed Sept. 3, 1957, Ser. No. 681,434  
13 Claims. (Cl. 44—66)

The invention relates to improvements in the suppression of surface ignition and reduction of octane requirement increase of leaded fuels in the operation of spark-ignition internal combustion engines. More particularly, this invention provides leaded fuels containing novel additives which are effective in suppressing surface ignition and reducing octane requirement increase.

It is known that the presence of organolead antiknock agents, such as tetraethyllead, in the fuel burned in a spark-ignition internal combustion engine leads to the formation of combustion chamber deposits which are detrimental to the efficient operation of the engine. In spite of the use of lead scavenging agents, these deposits continue to grow in amount as the engine is operated until an equilibrium condition is reached in which the rate of formation of deposits equals the rate of removal in the exhaust gases and no further accumulation occurs. These deposits are harmful in that they cause an increase in the octane rating of the fuel needed for knock-free operation compared to that needed with the engine in a clean condition, which increase is known as the "octane requirement increase" (ORI) of the engine operating on the particular fuel. Another difficulty which is created by the presence of combustion chamber deposits from leaded fuels is surface ignition, i.e., the ignition of the fuel charge either before or after the passage of the spark caused by glowing of carbon deposits. Deposits from leaded fuels are largely responsible for this condition, since lead salts are known to lower the glow point of carbon.

It is an object of this invention to provide leaded fuel compositions for spark-ignition internal combustion engines which have a minimum tendency to promote surface ignition and increase octane requirement. A further object is to provide new and improved additives for addition to motor fuels for spark-ignition internal combustion engines in order to achieve these beneficial results.

I have discovered that the above objects can be achieved by providing a fuel comprising a major proportion of a hydrocarbon mixture boiling within the gasoline distillation range, minor amounts of an organolead antiknock compound and a halohydrocarbon lead scavenger, and an oil soluble mercury compound in an amount sufficient to reduce the susceptibility of the fuel to surface ignition, and preferably in an amount sufficient to give a mole ratio of mercury to lead in the fuel within the range from about 0.01 to about 1.0. In an advantageous embodiment the mercury compound, the halohydrocarbon scavenger, and the organolead antiknock compound are made up as a concentrate in a solvent oil vehicle. The concentrate may then be conveniently added in the required quantities to the hydrocarbon fuel before use, thus providing a finished fuel composition of the required octane rating which is inhibited against surface ignition and has a minimum tendency to increase the octane requirement of the engine.

In accordance with my invention there must be present in the combustion chamber of an engine operated on a leaded fuel a small but effective proportion of a mercury compound. Although any practicable method of introducing the mercury compound into the combustion chamber can be used, as by injecting it in solution as a sepa-

## 2

rate stream, it is most convenient and thus the preferred embodiment of the invention, to dissolve the mercury compound in the fuel. The nature of the mercury compound does not appear to be controlling provided that it is sufficiently oil soluble for use in the fuel, since it is believed that under the conditions which obtain in the combustion chamber of the engine during use the same end product, probably mercuric oxide, results regardless of the original identity of the mercury compound. In 10 the course of my investigations, I have found that oil-soluble mercury salts of monocarboxylic acids are eminently suitable for use in my invention. Of these, mercury naphthenate and mercury oleate are particularly advantageous examples. Other useful mercury compounds, 15 by way of example, are soaps of mercury and fatty acids, such as mercury stearate, chelates of mercury and  $\beta$ -diketones, such as mercury acetylacetone, and mercury alkyl phenolates, such as mercury octyl phenolate. Whatever the mercury compounds used, it is preferred, although not essential, to use a sufficient amount in order to yield in the finished fuel composition a mole ratio of mercury to lead within the range from about 0.01 to about 1.0.

The lead antiknock compound which is used in this invention can be any of the organolead compounds which are useful for this purpose. By "organolead compound" is meant any compound in which the lead is directly linked to carbon atoms. Examples of suitable compounds are the lead aryls such as tetraphenyllead and the lead alkyls, particularly the tetra-alkyls, such as tetramethyllead, tetraethyllead, tetrapropyllead, tetrabutyllead, dimethyldiethyllead and the like, as well as mixtures of such compounds. Because of its availability and superior operating characteristics tetraethyllead is the preferred 35 organolead antiknock agent. It is customarily used at a concentration of about 0.5 cc. to 5.00 cc. per gallon of fuel.

The fuel compositions of my invention contain, as is customary with leaded fuels, the usual lead scavenging 40 compounds, the use of which is essential for satisfactory operation of the engine. These scavengers aid in the removal of much of the lead which would otherwise be deposited within the combustion chamber by combining with the lead to form volatile compounds which are removed in the engine exhaust gases. Scavengers are customarily halogenated hydrocarbons having about 2 to 8 carbon atoms and 2 to 3 or more halogen, especially bromine and/or chlorine, atoms per molecule. They are used in fuels in amounts of about 0.5 to 1.5 theories, a 45 theory being defined as the amount stoichiometrically required for reaction with the lead present in the fuel to produce the lead dihalide. Examples of suitable scavengers are ethylene dichloride, ethylene dibromide, trichloro-propane, chlorodibromobutane, trichlorocyclopentane, bromoethylbenzene and the like, as well as mixtures of these compounds. Ethylene dichloride and ethylene dibromide, which are in commercial use, are the preferred 55 scavengers for use in my invention.

The motor fuel used in this invention is preferably gasoline, but may be any other combustible liquid of suitable volatility commonly used as fuel for spark-ignition internal combustion engines, including paraffinic, naphthenic and aromatic hydrocarbons. The boiling point of such fuels should be in the range from about 100° F. to about 500° F., and preferably in the range from 150° F. to about 400° F. The fuel may also contain other ingredients commonly found in finished fuel compositions, such

as anti-oxidants, stabilizers, dyes, anti-icing agents and the like.

Although in most cases it will be found most convenient to add the mercury compounds of my invention to a finished fuel composition already containing the lead antiknock agent, it is also contemplated that an additive mixture be provided for addition to the fuel, which mixture contains the antiknock agent, tetraethyl lead for example, the halohydrocarbon scavenger, and the mercury compound in an amount to give a mole ratio of mercury to lead within the range of about 0.01 to about 1.0. The additive combination may be made up in any suitable solvent oil facilitating blending into the finished fuel, for example, naphtha, light gas oil, catalytic cycle oil, light lubricating oil fractions, or aromatic solvents such as benzene, toluene, xylenes and the like. Sufficient solvent oil should be used to provide desirable fluidity, for example, within the range of 25% to about 95% or more based on the total weight of the additive mixture. The additive combination may also contain desirable amounts of other common ingredients such as dyes, stabilizers, and the like.

Without being limited to any theory of the method by which the additives of my invention provide beneficial results, I believe these additives help in two ways to improve the operation of the engines to which they are used. The mercury compound may assist the halohydrocarbon scavenging agent in the removal of the combustion chamber deposits, thereby minimizing ORI and surface ignition caused by the deposits. In addition, the mercury compound may provide a catalytically active material which counteracts the tendency of the lead deposits which remain within the combustion chamber to promote the glowing of carbon particles. Thus, even in those instances when little or no reduction in combustion chamber deposits results from the use of the additives of my invention, there is nevertheless a decrease in ORI and surface ignition due to deposits.

As specific embodiments of my invention, the following examples are given. It is to be understood that these are by way of illustration only and are not intended as a limitation of my invention.

#### EXAMPLE I

A test was made in which an air-cooled, single cylinder Lauson engine was operated on a fuel containing TEL, ethylene dichloride and ethylene dibromide scavengers, and one of the mercury compounds of my invention, specifically mercury naphthenate. Combustion chamber deposit weights obtained using this fuel were compared with those obtained with the same fuel from which the mercury naphthenate was omitted. The operating conditions were 50 hours at 50 watt steady load and 1800 r.p.m. Results were as follows:

#### Combustion Chamber Deposit Weight (g)

|                          | Base Fuel <sup>1</sup> | Base Fuel+.0375% Mercury Naphthenate | Mole Ratio, Hg/Pb | Percent Reduction in Deposit Weight |
|--------------------------|------------------------|--------------------------------------|-------------------|-------------------------------------|
| Lauson Engine No. 1----- | 5.80                   | 3.95                                 | 0.1               | 32                                  |
| Lauson Engine No. 2----- | 6.14                   | 3.66                                 | 0.1               | 40                                  |

<sup>1</sup> Gasoline containing 3 cc. TEL/gal., 1.0 theory of ethylene dichloride, and 0.5 theory of ethylene dibromide.

As can be seen from the above data the presence of the mercury naphthenate resulted in a reduction in deposit weight of 30 to 40%.

#### EXAMPLE II

The benefits obtained in using the additives of my invention were further demonstrated by the results obtained

in a CFR overhead valve engine in 165-hour cycled runs under the following conditions:

|                                                   | Cycle |      |
|---------------------------------------------------|-------|------|
| 5                                                 |       |      |
| Compression Ratio, 6.4—Load-----                  | None  | Full |
| Coolant Temp., ° F., 148±3—Time, sec-----         | 45    | 135  |
| Oil Temp., ° F., 160±5—Speed, r.p.m-----          | 900   | 900  |
| Intake Air Temp., ° F., 110±5—Air/Fuel Ratio----- | 12.5  | 13.0 |

10 Results were as follows:

|                                        | Base Fuel <sup>1</sup> | Base Fuel+.0375% Hg Naphthenate <sup>2</sup> | Percent Reduction |
|----------------------------------------|------------------------|----------------------------------------------|-------------------|
| 15 Octane Requirement Increase-----    | 12.5                   | 5.0                                          | 60.0              |
| Surface Ignition, Counts per Hour----- | 366                    | 266                                          | 27.3              |

<sup>1</sup> Gasoline containing 3 cc. TEL/gal., 1.0 theory of ethylene dichloride, and 0.5 theory of ethylene dibromide.

<sup>2</sup> Mole ratio Hg/Pb=0.1.

20 These data illustrate the marked decrease in deposit harm, as evidenced by the large reduction in octane requirement increase and surface ignition, which results from the use of the additives of my invention.

#### EXAMPLE III

Further tests with a 17.6 D.C. single cylinder engine again demonstrated the reduction in ORI which follows from the use of the mercury compounds of this invention. The tests used in each case were 165 hour cycled runs carried out under the following conditions:

|                                                    | Cycle |      |
|----------------------------------------------------|-------|------|
| 30                                                 |       |      |
| Compression Ratio, 7.7—Load-----                   | None  | Full |
| Coolant Temp., ° F., 148±3—Time, sec-----          | 45    | 135  |
| Oil Temp., ° F., 160±5—Speed, r.p.m-----           | 900   | 900  |
| Intake Air, Temp., ° F., 110±5—Air/Fuel Ratio----- | 12.5  | 13.5 |

40 Results were as follows:

|                                     | Base Fuel <sup>1</sup> | Base Fuel+.0375% Hg Naphthenate <sup>2</sup> | Percent Improvement |
|-------------------------------------|------------------------|----------------------------------------------|---------------------|
| 45 Octane Requirement Increase----- | 14.5                   | 5.0                                          | 66                  |

<sup>1</sup> Gasoline containing 3 cc. TEL/gal., 1.0 theory of ethylene dichloride and 0.5 theory of ethylene dibromide.

<sup>2</sup> Mole ratio Hg/Pb=0.1.

50 As can be seen in this example, an outstanding reduction in ORI was achieved by the addition to the fuel of 0.0375% mercury naphthenate. Results similar to those of this and the other examples can be obtained with other oil soluble mercury compounds, such as mercury oleate, mercury stearate, mercury acetylacetone, and the like.

#### EXAMPLE IV

60 The effectiveness of the mercury compounds of my invention is further demonstrated by the results obtained on 150 hour cycled runs with a 1953 Pontiac 8-cylinder engine. The runs were carried out under the following conditions.

| 65 Cycle----- | Duration-----  | 45 sec-----      | 135 sec----- | Once an hour a 2,000 r.p.m. wide open throttle acceleration for 30 sec. |
|---------------|----------------|------------------|--------------|-------------------------------------------------------------------------|
| Engine Speed. | 700 r.p.m----- | 2,000 r.p.m----- |              |                                                                         |
| Load-----     | None-----      | 26 lbs-----      |              |                                                                         |

70 Compression ratio—7.6:1,  
Air/Fuel ratio—As found,  
Coolant temp.—160±5° F.,  
Oil temp.—165±5° F.

The addition of mercury naphthenate to the fuel caused a significant decrease in the amount of combustion cham-

ber deposits formed and in the octane requirement increase as can be seen from the following results:

|                             | Base Fuel <sup>1</sup> | Base Fuel + 0.0375% Hg Naphthenate <sup>3</sup> | Percent Improvement |
|-----------------------------|------------------------|-------------------------------------------------|---------------------|
| Deposit Wt. (g.)            | <sup>2</sup> 85.6      | 68.5                                            | 20                  |
| Octane Requirement Increase | <sup>2</sup> 3.8       | 3.0                                             | 21                  |

<sup>1</sup> Gasoline containing 3 cc. TEL/gal., 1.0 theory of ethylene dichloride and 0.5 theory of ethylene dibromide.

<sup>2</sup> Average of three tests.

<sup>3</sup> Mole ratio Hg/Pb=0.1.

In evaluating new additives it is important to determine whether or not they have any harmful effect on such fuel properties as stability and octane number. The results of the tests shown in the following table indicate that the additives of my invention have no adverse effects in this respect.

TABLE I

|                                                                        | Induction Period (min.) <sup>1</sup> | Octane Rating (Research) |
|------------------------------------------------------------------------|--------------------------------------|--------------------------|
| Gasoline A (3.0 cc. TEL/gal., 1.5 theories halohydrocarbon scavengers) | 455                                  | 92.2                     |
| Gasoline A+0.0375% Hg naphthenate (mole ratio Hg/Pb=0.1)               | 420                                  | 92.2                     |

<sup>1</sup> ASTM D525-49.

While I have described my invention by reference to specific embodiments thereof, the same are given by way of illustration only. Modifications and variations will be apparent from my description to those skilled in the art.

I claim:

1. A fuel composition for a spark ignition internal combustion engine comprising a major proportion of a hydrocarbon mixture boiling within the gasoline distillation range, from about 0.5 to about 5.0 cc. per gallon of fuel of an organolead antiknock compound, from about 0.5 to about 1.5 theories of a halohydrocarbon scavenger, and an oil soluble mercury compound capable of forming mercury oxide under spark ignition internal combustion engine combustion chamber conditions, said mercury compound being present in an amount sufficient to reduce the susceptibility of said fuel composition to surface ignition.

2. The fuel composition of claim 1 in which said mercury compound is mercury naphthenate.

3. The fuel composition of claim 1 in which said mercury compound is mercury oleate.

4. The fuel composition of claim 1 in which said antiknock compound is tetraethyllead.

5. A fuel composition for a spark ignition internal combustion engine comprising a major proportion of gasoline, tetraethyllead in an amount from about 0.5 to about 5.0 cc. per gallon of gasoline, from about 0.5 to about 1.5 theories of a halohydrocarbon lead scavenger, and an oil soluble mercury compound capable of form-

ing mercury oxide under spark ignition internal combustion engine combustion chamber conditions, said mercury compound being present in an amount sufficient to give a mole ratio of mercury to lead in the range from about 0.01 to about 1.0.

6. A fuel composition for a spark ignition internal combustion engine comprising a major proportion of gasoline, tetraethyllead in an amount from about 0.5 to about 5.0 cc. per gallon of gasoline, from about 0.5 to about 1.5

10 theories of a halohydrocarbon lead scavenger, and an oil soluble mercury salt of a monocarboxylic acid in an amount sufficient to give a mole ratio of mercury to lead in the range from about 0.01 to about 1.0.

7. The fuel composition of claim 6 in which said mercury salt is mercury naphthenate.

8. The fuel composition of claim 6 in which said mercury salt is mercury oleate.

9. An additive combination for gasoline consisting essentially of an organolead antiknock compound, from about 0.5 to about 1.5 theories of a halohydrocarbon lead scavenger, and an oil soluble mercury compound capable of forming mercury oxide under spark ignition internal combustion engine combustion chamber conditions, said mercury compound being present in an amount sufficient

25 to give a mole ratio of mercury to lead in the range from about 0.01 to about 1.0.

10. The additive composition of claim 9 in which said organolead antiknock compound is tetraethyllead.

11. The additive composition of claim 9 in which said 30 mercury compound is mercury naphthenate.

12. The additive composition of claim 9 in which said mercury compound is mercury oleate.

13. In a spark ignition internal combustion engine using a hydrocarbon fuel containing an organo-lead anti-35 knock composition and a halohydrocarbon scavenger the method of reducing octane requirement increase and surface ignition in the combustion chamber of the spark ignition internal combustion engine which comprises introducing oxygen and an oil-soluble mercury compound 40 capable of forming mercury oxide under spark ignition internal combustion engine combustion chamber conditions in the presence of said hydrocarbon fuel containing from about 0.5 to about 5.0 cc. per gallon of fuel of an organo-lead antiknock composition and from about 0.5 to about 1.5 theories of a halohydrocarbon scavenger into the combustion chamber.

References Cited in the file of this patent

UNITED STATES PATENTS

|              |               |               |
|--------------|---------------|---------------|
| 1,841,254    | Rosenbaum     | Jan. 12, 1932 |
| 2,151,432    | Lyons et al.  | Mar. 21, 1939 |
| 2,258,297    | Miller et al. | Oct. 7, 1941  |
| 2,314,575    | Doran         | Mar. 23, 1943 |
| 55 2,356,476 | Shappirio     | Aug. 22, 1944 |
| 2,364,921    | Shokal        | Dec. 12, 1944 |
| 2,671,758    | Rubin et al.  | Mar. 9, 1954  |
| 2,926,184    | Irish et al.  | Feb. 23, 1960 |
| 2,933,380    | Kegelman      | Apr. 19, 1960 |